

## UNITED STATES PATENT OFFICE

JULIUS EISELE, ROBERT GRIESSBACH, AND CLAUS HEUCK, OF LUDWIGSHAFEN-ON-THE-RHINE, GERMANY, ASSIGNORS TO I. G. FARBNINDUSTRIE AKTIENGESELLSCHAFT, OF FRANKFORT-ON-THE-MAIN, GERMANY, A CORPORATION OF GERMANY

## FOAM FLOTATION

No Drawing. Application filed February 9, 1928, Serial No. 253,214, and in Germany February 16, 1927.

The foam flotation process for the preparation of coal, ores, slags and the like and more especially for the separation of inferior coals and low-grade ores from ash constituents, 5 impurities and gangue, is carried out with flotation agents, which should have the property, on the one hand, of effectually wetting the material to be floated, and, on the other, of generating foam. The flotation agents hitherto employed for this purpose, such as 10 paraffins, tars, phenols and aromatic amines, combine these two properties only imperfectly if at all, and for this reason the addition of special foam producers, such as pine oils, 15 crude turpentine, saponins, sulfonic acids or salts of same, and the like is required.

We have found that the products obtained by oxidizing hydrocarbons more especially 20 paraffins, or waxes and the like at comparatively low temperatures, generally not exceeding 200° C., so that no decomposition occurs, can be employed to great advantage as flotation agents. These substances possess the property of floating coal and ores and especially sulfid ores, in aqueous suspensions, so 25 that a considerable concentration of high-grade coal or ore is obtained in the foam. These products also act as powerful foaming agents, and it is therefore unnecessary 30 to add any further foam producers. Most of the said oxidation products contain free carboxylic acid groups which are preferably neutralized, more or less completely, with bases such as ammonia.

The following examples will further illustrate the nature of the said invention which however is not limited thereto.

## Example 1

40 Finely ground brown-coal, or brown-coal dust, with over 23 per cent of ash content in proportion to the dry substance, is treated by the flotation process in a conically shaped apparatus of any known kind, air being 45 passed through. The flotation agent added consists of a readily volatile oxidation product of paraffin wax, neutralized with ammonia, the amount employed being 1 per cent of the weight of dry substance in the material treated. After a short treatment, the

resulting coal concentrate is drawn off, and its ash content is found to have been reduced by more than 50 per cent.

## Example 2

55 A difficultly volatile oxidation product of Montan wax, neutralized with ammonia, is employed as a flotation agent in the manner described in Example 1. In this case also, the original ash content of the coal is reduced to less than one half.

## Example 3

Sandy pyrites is subjected to flotation by adding a difficultly volatile, neutralized oxidation product of paraffin wax, the amount of the agent being 1 per cent the weight of the ore. The pyrites content in the foam is three times that originally present in the sandy pyrites.

## Example 4

75 Finely ground brown-coal with a content of 46 per cent of ashes in proportion to the dry substance is subjected to flotation after admixing a difficultly volatile oxidation product of paraffin wax in an amount of 1 per cent of the dry weight of the brown-coal to be treated. After a short treatment a concentrate of coal is drawn off, the content of ashes 80 of which amounts to only 16 per cent of the dry substance.

What we claim is:

1. The process of foam flotation, which comprises intensely mixing an aqueous pulp 85 of the material to be treated with a product of the oxidation at an elevated temperature not exceeding 200° C. of a material, comprising hydrocarbons of high molecular weight, then passing a current of a gas through the mixture and separating the resulting froth.

2. The process of foam flotation, which comprises intensely mixing an aqueous pulp 90 of the material to be treated with a product of the oxidation at an elevated temperature not exceeding 200° C. of a material comprising paraffin wax, then passing a current of a gas through the mixture and separating the resulting froth.

3. The process of foam flotation, which 100

comprises intensely mixing an aqueous pulp of the material to be treated with a product of the oxidation at an elevated temperature not exceeding 200° C. of a material mainly consisting of hydrocarbons of a high molecular weight, and with an amount of a basic agent at the most equivalent to the quantity of free acids contained in the said oxidation product, then passing a current of air through 10 the resulting mixture and separating the resulting froth.

4. The process of foam flotation, which comprises intensely mixing an aqueous pulp of the material to be treated with a product 15 of the oxidation at an elevated temperature not exceeding 200° C., and with ammonia, then passing a current of a gas through the resulting mixture and separating the resulting froth.

20 5. The process of foam flotation, which comprises intensely mixing an aqueous pulp of the material to be treated with about 1 per cent its weight of a product of the oxidation at an elevated temperature not exceeding 200° 25 C. of paraffin wax, and with a quantity of ammonia exactly neutralizing the free acids contained in the said oxidation product, then passing a current of air through the resulting mixture and separating the resulting froth.

30 In testimony whereof we have hereunto set our hands.

JULIUS EISELE.  
ROBERT GRIESSBACH.  
CLAUS HEUCK.

35

40

45

50

55

60

65